

1,027,165.

H. I. WOOD.  
METHOD OF TREATING FILAMENTS.  
APPLICATION FILED FEB. 9, 1907.

Patented May 21, 1912.



Witnesses:

Marcus L. Byng  
W. Ray Taylor.

Inventor:  
Howard I. Wood,  
By *Alfred H. Davis*  
Atty.

# UNITED STATES PATENT OFFICE.

HOWARD I. WOOD, OF SCHENECTADY, NEW YORK, ASSIGNOR TO GENERAL ELECTRIC COMPANY, A CORPORATION OF NEW YORK.

## METHOD OF TREATING FILAMENTS.

1,027,165.

Specification of Letters Patent. Patented May 21, 1912.

Application filed February 9, 1907. Serial No. 356,559.

To all whom it may concern:

Be it known that I, HOWARD I. WOOD, a citizen of the United States, residing at Schenectady, in the county of Schenectady 5 and State of New York, have invented certain new and useful Improvements in Methods of Treating Filaments, of which the following is a specification.

My present invention relates to the manufacture of incandescent lamp filaments, particularly filaments of high fusing metal such as tungsten, molybdenum, titanium, by the use of a vaporizable binder, and its object is to render the process of manufacture more expeditious and cheaper, to decrease the breakage of the filaments in carrying out the process, and to improve it in other particulars.

The invention comprises an improvement 20 in the process of filament manufacture invented by William D. Coolidge, and contemplates a novel apparatus for carrying out certain steps of the treatment.

The Coolidge process, above referred to, 25 consists in mixing powdered metal such as tungsten, with a ductile binding means, such as warm cadmium amalgam, heating the mixture to a plastic condition, and then extruding the mixture so formed to produce 30 ductile wires. These wires are then treated to drive out the mercury and cadmium. A coherent body of the refractory metal is left behind. A mixture suitable for this treatment consists of equal parts mercury and 35 cadmium, to which is added 39% by weight of powdered tungsten. A simple method of driving out the mercury and cadmium consists in passing an electric current through the ductile wire while in a vacuum, and 40 thereby heating it up to the temperature at which the low fusing metals distil out. The filaments may then be heated to a much higher temperature to sinter the tungsten into a strong wire. Such a treatment, however, 45 must be given to the filaments individually and requires several seconds time for each filament.

According to my present invention, the 50 filaments are heated in a furnace to drive out substantially all the mercury, and possibly a small quantity of the cadmium, thereby reducing the time required for treating with current according to subsequent steps of the

Coolidge process. According to my invention the filaments are treated in quantities 55 of a hundred or more, simultaneously. The distillation of the volatile metal may, by my method, be carried on slowly and the slow distillation obviates the danger of flaws or of checks in the finished filaments. I do not 60 contemplate complete removal of the cadmium by my improved treatment, as such a proceeding would be liable to leave a residue 65 too fragile for commercial purposes. By taking out only the mercury, the cadmium remains to give the filament strength and 70 permit mounting in treating bottles, where current may be passed through to distil the cadmium and sinter the particles of tungsten together.

Not only does my invention decrease the time necessary for the production of a completed filament, but it also decreases the percentage of breakage during treatment. The wires of cadmium amalgam mixed with tungsten are initially quite strong and ductile, but when heated up to the temperature at which mercury distils, they become soft and somewhat delicate, and in fact, must, at this stage, be carefully handled. As soon, 80 however, as the mercury is all out, the filaments become strong again and may be handled without difficulty. When the filaments are baked in the furnace, according to my invention, they pass through this delicate 85 stage while resting in bundles on the carbon boats, and they are therefore not subjected to any stresses tending to break or deform them. The bundles of filaments come out of the furnace with all the filaments intact and 90 the treatment is in a sense independent of the experience of the operator.

An apparatus suitable for carrying out my process is shown in the accompanying drawing, in which—

Figure 1 is an elevation of the vacuum furnace; Fig. 2 is a sectional view thereof; Fig. 3 is a diagram of the electrical connection of the electric heater, and Fig. 4 is a perspective view of the heater and of the 100 boats used to support the filaments in the furnace.

The vacuum furnace shown in Fig. 1 consists of a glass envelop 1 connected with a vacuum pump through a tube 2. The glass 105 envelop is provided with an end opening

closed by a suitable cap 3. Within this glass envelop is placed an electric heater 4 carrying carbon boats 5 on which the filaments are arranged in groups. Suitable connections 6 are provided for introducing current through the walls of a glass vessel to the conductors of the heater.

The electric heater consists of a plurality of iron coils 7 connected in parallel and inserted between sheets of mica 8. An aluminum plate 9 is arranged below the resistance coils and serves to hold them in place and also to thermally insulate the coils from the lower wall to the glass envelop. The carbon or graphite boats 5 are provided with longitudinal grooves 10 in which the looped filaments 11 are arranged. A heavy copper plate 12 is interposed between the boats and the hot coils and serves to equalize the heat on the boats and thereby insure uniform heating of the filaments.

In treating filaments according to my invention, the untreated wire of cadmium amalgam impregnated with tungsten is cut into suitable lengths for filaments, bent into loops and arranged in the carbon boats as shown in Fig. 4. Several of these boats are then introduced into the furnace, as shown in Fig. 1, and the cap 3 is placed on the end of the furnace and the furnace chamber is evacuated. Current is then supplied to the resistance coil 7 and the temperature within the furnace is slowly raised until the distillation of mercury is effected. A temperature of 215° C. gives good results, but a more rapid distillation may be effected by running the furnace at a somewhat higher temperature. At present I believe that some cadmium comes off with the mercury even at temperatures below the normal vaporizing point of cadmium, but sufficient cadmium remains in the filaments to render them strong and suitable for ready manipulation according to subsequent steps of the Coolidge process. When a temperature of about 215° is used the heat treatment may be continued for a period of 60 minutes. The filaments are then allowed to cool, and after removal from the furnace are separated and treated individually with current as in the original Coolidge process. This current drives out the remaining vaporizable components and sinters together the tungsten particles into a strong coherent filament. The use of my invention in conjunction with other steps of the Coolidge treatment so shortens the work and decreases the breakage that the output of filaments, for a given number of operators, may be increased fully four fold.

What I claim as new and desire to secure by Letters Patent of the United States, is,

1. As a step in the production of metal filaments, the process which consists in bak-

ing wire of cadmium-amalgam impregnated with tungsten to drive out mercury and leave a coherent conductor containing cadmium and tungsten.

2. As a step in the production of metal filaments, the process which consists in baking an unfinished filament rendered coherent by the presence of metallic material comprising mercury and more refractory metal *in vacuo* to drive mercury therefrom.

3. As a step in the production of metal filaments, the process which consists in baking a composite wire rendered coherent by the presence of vaporizable metal to drive an easily vaporizable portion of such metal therefrom, and then heating said wire with current to drive an additional portion of vaporizable metal therefrom and sinter the residue.

4. As a step in the production of lamp filaments from a mixture of refractory metal and metallic material comprising a plurality of low melting metals, the process which consists in baking the mixture to drive out a less refractory portion of said material and thus produce filament shaped conductors which may subsequently be treated to drive out the remainder of said material and yield filaments of pure tungsten.

5. The process which consists in baking wires comprising a refractory powder incorporated in an amalgam containing vaporizable material to drive mercury therefrom, and subsequently passing current through said wires to drive out any easily vaporizable material and sinter the residue into a coherent refractory conductor.

6. The process of treating a composite conductor composed of refractory metal powder held by a less refractory alloy, which consists in heating the wire by external means to drive out part of the material of said alloy, then heating said wire with current passed therethrough to drive out the remainder of said alloy, continuing the heating to sinter the final residue into a coherent refractory conductor suitable for lamp filaments.

7. As a step in the production of refractory conductors, the process which consists in treating by radiant heat a filamentary body, composed of highly refractory metal held together by a binder having components of different degrees of refractoriness, so as to expel a component of the binder of low refractoriness, and then passing an electric current through said body to heat it to a higher temperature, so as to expel the rest of the binder and leave only the pure metal and to sinter the highly refractory residue.

8. As a step in the production of filaments, the process which consists in baking a filamentary body containing highly re-

refractory material and metallic material of relatively low refractoriness by the presence of which it is rendered coherent to expel a portion of the latter and produce a conductor consisting of highly refractory material and a more refractory portion of said latter.

In witness whereof, I have hereunto set my hand this 7th day of February, 1907.

HOWARD I. WOOD.

Witnesses:

BENJAMIN B. HULL,  
HELEN ORFORD.